

Feb. 2, 1937.

H. G. NEVITT

2,069,620

METHOD FOR MANUFACTURING RESIDUAL OILS OF HIGH ASPHALTIC CONTENT

Filed June 16, 1932

*Fig. 1*



*Fig. 2*



INVENTOR

*Henry G. Nevitt*

BY

*Dallas R. Lamont*

ATTORNEY

## UNITED STATES PATENT OFFICE

2,069,620

METHOD FOR MANUFACTURING RESIDUAL  
OILS OF HIGH ASPHALTIC CONTENTHenry G. Nevitt, Kansas City, Mo., assignor to  
Socony-Vacuum Oil Company, Incorporated,  
New York, N. Y., a corporation of New York

Application June 16, 1932, Serial No. 617,529

4 Claims. (Cl. 196—74)

This invention relates to the manufacture of residual hydrocarbon oils of highly asphaltic nature such as are used for binders in the construction of oiled and asphaltic road surfaces 5 and for other construction and manufacturing uses for which products of this type are adapted.

Specifically it relates to method and means for manufacturing the desired product from raw materials, and to method and means for separating such product where it occurs in recoverable form in residual streams from other processes which may be operated for other purposes.

Asphaltic road oils are essentially oils of an asphaltic or asphalt-like nature diluted to a greater or less degree with lighter oils of a semi-asphaltic or non-asphaltic nature. The degree of dilution is that required to meet specifications as to asphalt content, viscosity, and the like. Ductility and percentage of free carbon in the residue are also frequently specified. In use, these oils fulfill varying purposes ranging from the compacting and water-proofing of dirt roads to the production, when mixed with gravel, of a high type of surface approaching bituminous concrete in nature. Due to the necessarily wide range of specifications, which arises both from range of application and from lack of precise knowledge of the meaning of specific properties, a rigorous definition of road oil can not be formulated.

To those acquainted with the art, the term "asphaltic road oil" has a definite meaning. This meaning is more physical than chemical, and while the range of the class is wide, it is realized within the art that materials of this class are distinctly different from ordinary fuel oil residues produced at random conditions. It is equally well realized that mere reduction of an ordinary fuel oil residue to meet specifications of penetration or of viscosity will rarely result in a road oil meeting other specifications which are equally important except by the fortuitous circumstance of the starting material having been fit for the product. The manufacture of road oils is essentially a manufacture in that proper starting materials must be selected and proper process steps carried out upon them in order that the final product shall fully meet all of the desired specifications. The mere reduction or dilution of any residue to meet one point of specification usually results in a failure to adequately meet most of the other points of specification.

As an example of the type of material at present designated as road oil, there is quoted here the official specification adopted for one

type of road oil by the Highway Department of the State of Nebraska for the year 1931.

## Nebraska 1931 road oil specifications

(Adopted April 1, 1931)

| A. Type of oil                                                             | No. 1 Road Oil for<br>Sand-Hill Constr. |      | 10 |
|----------------------------------------------------------------------------|-----------------------------------------|------|----|
|                                                                            | Min.                                    | Max. |    |
| Viscosity (Saybolt furol) 122° F., seconds                                 |                                         | 500  |    |
| Asphalt residue of 100 penetration (77° F.)<br>percent                     | 75                                      |      |    |
| Ductility of asphalt residue at 77° F.,<br>cms.                            | 75                                      |      |    |
| Flash point (Cleveland open cup), degrees<br>F.                            | 200                                     |      | 15 |
| Specific gravity at 77/77° F.                                              | 1.040                                   |      |    |
| Volatilization loss (325° F., 50 gms., 5 hrs.)<br>per cent                 |                                         | 4    |    |
| Distillation test;<br>Total percent distilled up to 680° F.<br>(sea level) |                                         | 3    | 20 |
| Bitumen insoluble in 86° Baumé naphtha,<br>percent                         | 14                                      |      |    |
| Soluble in carbon tetrachloride, percent                                   | 99.50                                   |      | 4  |
| Paraffin wax or scale, per cent                                            |                                         | 4    |    |
| Water and sediment, per cent                                               |                                         | 2    |    |

This oil is one which has been successfully used for the purpose intended, and can be produced with ease by the method set forth in the present disclosure. The production of this material by the methods of the prior art, with which I am at present familiar, is a matter of considerable difficulty and usually to meet some of the specifications requires that some of the others be disregarded.

Other products of the same general type which may be manufactured by the process of this invention and are within the contemplation of this invention run throughout the range from very dilute to extremely concentrated residues, many of which may be solid or semi-solid at atmospheric temperatures. All of these products, however, will show in varying degrees the physical properties characteristic of the type.

The starting material for road oil manufacture will usually be an oil containing asphaltic material, and such asphaltic material may be either of natural origin or the result of previous treatment of the oil. When the starting material is residual oil from an asphalt base or mixed base crude the asphaltic material is of natural origin. Frequently the asphaltic material has originated as a result of some prior treatment of the oil. For instance the oil may have been oxidized or treated with sulphur with the definite aim of producing asphalt-like material. Also, the asphaltic

material is frequently present as the result of cracking, or some other prior step which was not carried out with the intention of producing asphalt, and is in effect a by-product.

- 5 Usual commercial methods of producing such asphaltic residual oils of which I am aware consist generally of batch processes. These starting materials above-mentioned are placed in shell stills, heated to vaporize light fractions and reduced to the desired consistency. An alternate method is to heat the starting material in a pipe coil heater and "flash" to the required residue. Either of these methods requires a reheating which is not only in itself costly, but which is 10 more or less incapable of that rigid control which is necessary to avoid side reactions resulting in the reduction of viscosity of the desired residue or formation of "free carbon", both of which are detrimental to the product.
- 15 20 Materials of an asphaltic nature are present in the residual oils of most commercial cracking systems. As a usual case, the usefulness of these oils is decreased due to the manner in which they are separated from the process. A prolonged exposure to the heat and pressure conditions of cracking results in decomposition with alteration of the viscosity and ductility usually associated with a given specific gravity, and in an increase in "free carbon" insoluble in the usual test solvents. In consequence of this the ordinary residual oils from cracking operations are usually very 25 far from the characteristics required in good road oils.
- 30

I have found that by the process of my invention as herein disclosed I may separate the asphaltic residual oils, no matter from what source, in such a manner as to prevent their decomposition and preserve in them all of the inherent characteristics of the starting stock which would tend 35 to make a good road oil. I have also found that this process enables me to operate in connection with processes which produce an asphaltic residue, but normally decompose it or contaminate it, in such a manner as to "rescue" the asphaltic material from the system with a minimum of decomposition or contamination. I have thus been 40 able to avail myself of a considerably wider source for the production of road oils of superior quality 45 than is at present known to the industry.

50 55 I have also found that the process of this invention, when operated in conjunction with other processes such as cracking processes, enables me to separate the asphaltic oils in a manner which does not in any way interfere with the proper operation of the system from which they originate 60 for its principal purpose. Also, by the process of the invention I am enabled to separate the operation of parting the asphaltic materials from the system from the operation of generating the asphaltic materials so that each step in the operation 65 may be operated with a maximum of efficiency.

This invention has for an object the provision of a method for separately controlling the production 65 conditions for the asphaltic material and the final specifications of the finished product in order that one may be varied as desired without materially affecting the other.

A further object is the provision of apparatus in 70 which the process of the invention may be carried out.

A further object of this invention is that of 75 enabling the adaption of existing processes for cracking and/or synthesizing gasoline in such manner that their residual oils may be so sep-

arated as to yield an asphaltic oil of desirable characteristics.

Among the objects of this invention are those of controlling the chemical characteristics of the product, controlling the physical characteristics 5 of the product, controlling the character of the stock from which the product is synthesized or segregated and such further objects as may hereinafter appear.

In principle the method of this invention consists of two parts. The first, generally applicable to any condition under which asphaltic materials may originate, contemplates their removal from such system in a manner which will minimize the effect of continuing decomposition under the conditions of that system. The second contemplates the selection of the stock which is removed, the selection of the diluent stock, and the selection of the stock which is returned in such manner that both the problem of meeting specifications of 20 product and the problem of best operation of the originating system are commercially met.

In order that the method and apparatus by which my invention is practised may be more thoroughly understood, reference is made to the 25 drawing attached to and made a part of this specification.

Figure 1 illustrates in diagrammatic form the application of my invention to cracking processes where cracking is completed within the heating 30 coil followed by vaporization and separation. The vaporizer of the cracking system in this case may be fitted to carry out my invention without in any way disturbing its normal function as an integral portion of the cracking system. Figure 1 35 may also be considered to set forth a system which can be used primarily for the production of asphaltic residue with cracking as an incidental thereto, as hereinafter explained.

Figure 2 illustrates an apparatus which has 40 been successfully used in the practice of the invention.

Referring more specifically to Figure 2, A is a vaporizing chamber shown in section in order that internal arrangements may be made clear. 45 This vaporizing chamber may or may not be fitted in its upper portions with baffles, mist-catching devices, or bubble trays, the presence or absence of these being more or less optional as required by the process in conjunction with 50 which this vaporizer is operated. However, it is intended that the function of the body A should be basically that of a vaporizer and any fractionation as by extensive use of bubble trays, etc., should not be considered a portion of the duty 55 of this body A and except as necessary for the removal of mist, etc., return to the liquid in the bottom of body A of any material condensed in the upper portion preferably should not be practised.

Entering the side of the vaporizer A at a point spaced above its bottom is a pipe 1 equipped with a valve. The purpose of this pipe is to introduce into the vaporizer the stream of products to be vaporized and separated therein. The 65 valve upon this line may be merely for the purpose of cutoff or it may be required by the system in which the vaporizer is operated as a controller valve of that system. That is to say, the valve is not a necessary feature of pipe 1. At the 70 top of the vaporizer A vapors are allowed to pass out through pipe 2. At the bottom of the vaporizer A, there is provided storage for a small amount of unvaporized residue. This residue is allowed to pass from the vaporizer A through line 75

4. The level of this liquid is maintained at some point such as 5, by automatic or manual control of a valve placed in line 4. Line 3 enters the side of the vaporizer and discharges at some point between line 1 and liquid level 5 through a spray device as indicated, or if preferred, it may discharge below liquid level 5 in the bottom of the liquid. In operation the function of this line 3 is to introduce into the vaporizer A an oil 10 substantially unheated or heated partially to its temperature of vaporization in order that by vaporizing within the vaporizer it may extract sufficient heat to cool the residue unvaporized from the stream entering through line 1 and thereby control the physical characteristics of 15 the material drawn off through line 4.

Other and concurrent functions of the stream entering through pipe 3 are mentioned elsewhere in this specification. Referring now to Figure 1, A is the vaporizer as before and 1, 2, 3, 4 and 5 have the same meaning as before expressed. B is a bubble tower, C a furnace and D a pump. This system illustrates the use of my invention in connection with cracking processes 25 wherein the reaction is complete within the heating coils. In this process the pump D, taking suction from the bottom of the bubble tower B, passes the oil through coils in furnace C. Such oil may or may not be under pressure in 30 excess of that required to overcome flow resistance.

In case back pressure is held upon the heating coil, it may be released through the valve in line 1. Entering vaporizer A the reaction stream 35 from line 1, consisting of cracked products, uncracked and unpolymerized gas oil, partially polymerized gas oil, and polymerized residue separates, the polymerized residue falling to the bottom to be removed to storage and the cracked 40 product, unconverted gas oil and partially polymerized gas oil pass through vapor line 2 to bubble tower B. In this bubble tower the portions heavier than the cracked products are condensed to be collected in the bottom and returned 45 to the furnace by pump D.

The cracked products pass over-head from the bubble tower to be condensed and taken to storage. Charge for the system is introduced from a storage tank into the bubble tower. Gas 50 oil taken from a storage tank is discharged into vaporizer A through line 3 and the asphaltic residue product is withdrawn through line 4. In the operation of this system, the temperature of vaporizer A at and above the entrance of line 1 is so controlled that partially polymerized products of the reaction stream remain as vapors and only such products of the reaction stream as are 55 of satisfactory nature remain unvaporized to collect in the storage below liquid level 5. To 60 check further evaporation from and/or change in this product in the short time interval that must elapse before it can be withdrawn the cooling effect of oil from line 3 is taken advantage of. It may also be the case that some portion 65 of the oil from line 3 remains unvaporized to join with the asphaltic residue and it is in the inter-relation of the temperatures at the entrance level of line 1 and below liquid level 5 as controlled by the amount of oil introduced 70 through line 3 that the final characteristics of the product withdrawn through line 4 are controlled.

In another sense the apparatus of Figure 1 may be considered as a method for making asphalt residue rather than as a method for mak- 75

ing a cracked product of the nature of gasoline. That is to say, the system of Figure 1, of which vaporizer A is a part, is of such a nature that its operation in the method described above but with variations in the stock primarily charged, time 5 relation of various elements, etc., could be operated for the production of an asphalt residue with the production of gasoline-like hydrocarbons incidental thereto.

It is understood as the sense of above discussion that this invention may be applied, not only to the specific process as above related, but that it may be applied to processes of similar nature wherein the heating coil, with or without back pressure, is followed by vaporizer operation to 10 separate from the reaction stream the heavy product formed therein. It is also to be understood that the process of this invention, insofar as it relates to the operation carried out in vaporizer A, as shown and explained in Figure 2 may 15 be carried out for the separation of asphaltic residual oil from a heated stream containing such asphaltic residue, regardless of its source. That is to say, the material entering the vaporizer may be the finished reaction stream of any process 20 designed to alter oils originally non-asphaltic to an asphaltic nature; it may be the residue portion of an asphaltic crude which has been subjected to topping and is desired to be further topped in the vaporizing body of this invention; or it may 25 be a stream of residual oil from any commercial cracking process, introduced to the vaporizer of this invention in order to separate from it asphaltic residual oil in the manner disclosed.

In the present process, if the apparatus of Figure 1 be used and the conditions chosen be such that the process of the main apparatus is that of cracking an oil to produce gasoline, the following discussion will be applicable; as in most cracking processes, the residual oil contains bodies of an 35 asphaltic nature.

The reaction stream entering through line 1 will have a temperature in the vicinity of 900° Fahrenheit and will consist of cracked gasoline product, uncracked gas oil, and products containing 40 varying amounts of asphalt or asphalt-like substances. Of these last, I prefer to retain only the heavier in liquid form, as they are of higher asphalt content. The others I desire to remain in the vapor state, both that I may 45 retreat them for the further production of asphaltic material and gasoline, and that they may not dilute my asphaltic base material which I am producing. To this end, I allow the vaporization at the entry point of pipe 1 to take place without 50 substantial drop in temperature other than that caused by the natural absorption of latent heat. To prevent the over-vaporization of the residue, to prevent its reaction with the formation of free 55 carbon, and to accomplish other corollary objects, it is desirable that the base residue be relieved of the influence of heat immediately.

It would be theoretically sufficient probably, to remove it immediately from its heated surroundings. Practically, this removal would be uncertain and at best would introduce a complication of apparatus. I prefer to cool it by spraying upon its surface; or introducing below its surface a stream of oil from pipe 3. This oil may be heated partially or almost to its vaporization point, 70 or it may be cold. Its heat content and amount are so adjusted that upon entering the vaporizer, it vaporizes and in picking up latent heat of vaporization cools the residue or base oil to a degree sufficient to prevent its continuing reaction 75

with deposition of carbon, etc. In cooling by this method I have a further advantage. If the residue produced under the best conditions for the system approaching the vaporizer be too heavy and viscous to meet specifications, as is usually the case, the amount of coolant can be so proportioned, or its properties can be so selected that a sufficient portion of it remains unvaporized and is hot blended with the base. Herein lies an important advantage of the process of my invention. The process which is producing the asphaltic residue, if its principal object is production of that residue, may be so adjusted as to get the maximum efficiency of yield and quality of base product. Then the alteration of the product to meet varying specifications can be conducted at will without affecting the adjustment of the process step where the product originates. If the process which is producing the asphaltic residue is a cracking operation, the desirable product may be separated and altered to meet specifications without impairing the maximum efficiency of the cracking process.

A further desirability of the process of my invention appears from consideration of the chemical theory at present believed to cover the facts. The reaction stream entering through line 1 consists of light gasoline-like hydrocarbons (present in varying quantity depending on whether or not the preceding process is one of cracking), unconverted gas oils, products partially polymerized to an asphaltic nature, and products polymerized sufficiently that they may be removed as asphaltic product.

Vaporization at high temperature, that is, without substantial extraction of heat, will render all except the last named vapor, leaving the desirable polymerized product as liquid. This product may be too heavy to meet physical specifications as to viscosity, etc., and must be cooled to avoid its further reaction which may result in formation of undesirable free carbon, loss of viscosity; etc. Virgin gas oil is admitted through line 3 and in vaporizing accomplishes the desired cooling.

The amount of gas oil so introduced and/or the temperature to which it is heated before introduction, in relation with the temperature of the vaporizer, governs the amount which may remain unvaporized to dilute the base oil to specification. In this way the lighter oils which are already partially polymerized are retained within the conversion cycle, with a resulting increase in efficiency for that cycle, and their place, insofar as their dilution function is concerned, is taken by virgin gas oil of similar physical characteristics, but of different chemical structure. The relationship between virgin gas oil hydrocarbons and partially polymerized hydrocarbons is such that for the same boiling point the partially polymerized product has a higher specific gravity and viscosity, and thus, solely by an operation broadly directed to heat regulation, the quality of product may actually be improved.

It is obvious to those skilled in the art that a general statement of temperatures, etc., would be of small value, due both to the varying characteristics of the process which is the source of the material entering through line 1, and to the broadness of the range of specifications which may be met by the material departing through line 4. With a given system or source of material and a given set of specifications to be met, it is possible for anyone skilled in the art using the disclosure of this invention to meet those specifications with no greater difficulty than is ordi-

narily encountered in adjusting any continuous process for controlled quality of product.

For instance, the product coming through the transfer line contains a certain percentage of asphalt capable of being separated as a product and has a certain temperature. The percentage of asphalt, as well as its characteristics, tends to vary greatly with the characteristics of the charging stock and cannot be predicted from any simple tests of the stock or deductions therefrom. A typical case would be an average mixed stock from a refinery operating on Mid Continent crude. At moderate pressures, if the transfer stream were not quenched the vaporizer top temperature would be about 780° F., the vaporizer bottom or liquid temperature would be about 760°, and the bottom product would be unfit for road oil of satisfactory quality. By introducing a quenching oil in the tower and reducing the bottom vaporizer or liquid temperature to preferably from 650° to 700° F., which can be done without materially affecting the vaporizing and other primary function operations of the unit, or giving an operation from such standpoint materially different from the first, I can produce a bottom product which has the following characteristics and is a desirable asphaltic product of its type.

*Specific gravity.*—Above 1.00, say 1.05 in typical case. 30

*Asphaltic content.*—Can be varied to suit by controlling reduction of residue in flash tower—say 70–80% in typical case.

*Viscosity.*—Can be varied to suit by controlling reduction of residue in flash tower—say, 300–600 seconds Saybolt furol @ 122° F. in typical case. 35

*Ductility of 100 penetration residue at 77° F.*—110 plus (relatively high at any penetration).

*Solubility in carbon tetrachloride and carbon disulphide.*—Relatively excellent—above 99.5% 40 in typical case.

*Insoluble in 86° paraffin naphtha.*—Relatively high—say 18% in typical case.

Similarly with other tests, which will show a very high quality product of its type, which cannot otherwise be made on this equipment from ordinary charging stocks without appreciably affecting the primary operation. 45

The quantity of quenching oil required in the bottom of the evaporator to reduce the temperature to the point in the range specified as determined by the requirements of the particular operation (or to not quite this range at some loss or risks of loss in quality characteristics in the road oil produced) evidently depends upon the proportion of road oil produced by the charging stock and upon the thermal characteristics of the quenching stock. The quantity can be calculated from the heat requirements of the cooling operation and the heat intake of the quenching stock when raised to the tower conditions. One advantage of my invention is the flexibility of this control, as small amounts of volatile quenching stock producing considerable cooling effect by vaporization, or larger amounts of less volatile quenching stock may be used to get the same thermal results. The choice will be dictated by operating conditions of the unit, degree of reduction, or other physical characteristics of the road oil produced due to the admixture of the non-volatile portion of the quenching stock to it, or other manufacturing reasons. 60

In the typical case referred to the per cent of road oil finally produced would be about 16% of the charging stock. The amount of quenching oil 70 75

used would be about 7 or 8% of the charge using the gas oil charge as quenching stock to cool the bottoms to around 660° F.

It may be seen that by the process of my invention I may produce oils of asphaltic nature under the conditions best suited for their manufacture, may separate from the stream only base oil of a desired nature, and return insufficiently treated oils to process; then, as a separately controlled step, I may bring about the dilution of the asphaltic material to a desired degree without in any way disturbing the conditions which I have found best for the production of the base oil.

Throughout this specification and in the following claims the terms "asphaltic" and "polymerized" have been used. These terms are here used in the general sense in which those terms are at present used in this branch of the industry. As this usage is considerably more loose and not specifically parallel to the general chemical significance of the terms the following explanatory definitions are made.

In the following claims where mention is made of "completely polymerized oil" it is intended that this term or its equivalent shall cover oil whose asphaltic content or asphalt-like nature is such that it may be withdrawn from the system as a desirable end product. Where "partially polymerized oil" is used, it is intended that this term or its equivalent shall cover oil whose nature is similar to the desired product yet which is not sufficiently so as to make it a desired end product, and which may be further altered to approach or become the desired end product.

It is also understood that the terms "asphaltic" and "asphalt-like" shall be synonymous in the interpretation of the claims and shall indicate an oil whose physical characteristics are of the kind generally understood as covered by the term asphaltic or meeting specifications of the kind noted, or capable of simple dilution or reduction to so meet them, regardless of actual chemical structure.

I claim:

1. That process of producing residual oil of high asphaltic content and low carbon content which comprises flowing a heated stream of oil containing an asphaltic residue into a vaporizing chamber, allowing vaporization under conditions of temperature and pressure not conducive to gasoline formation but capable of detrimental conversion of the asphaltic material to separate from that stream all products lighter than an asphaltic residue which contains 60-70 percent or more of 100 penetration asphalt, which has less than 1 percent of residue insoluble in carbon bisulphide, and which possesses physical properties suitable for road making material, cooling the said asphaltic residue to check further molecular structural change thereof, said cooling being accomplished by introducing to the vaporizer an oil which is substantially vaporizable at temperatures below that of the first vaporization, at a point without the main path of flow of vapors from said first vaporization, allowing said second oil to vaporize in contact with the residue from said first vaporization, and thereafter removing said asphaltic residue from the vaporizer.

2. That process of treating a heated stream of oil containing asphaltic material which comprises separating from it by vaporization under condi-

tions of temperature and pressure not conducive to gasoline formation but capable of detrimental conversion of asphaltic materials a heavy asphaltic residue, cooling the said residue to check further molecular structural change thereof by introducing to the vaporizer a second oil, said second oil vaporizing to a predetermined extent upon contact with said residue and prior to said contact having been protected from substantial contact with vapors from the first vaporization, and diluting the said residue with a selected unvaporized residue from said second oil to produce a combined residual oil containing at least 60-70 percent of 100 penetration asphalt, a carbon bisulphide insoluble portion of the order of 1 percent and possessing physical properties suitable for road making material.

3. That process of producing asphaltic residual oil which comprises establishing a stream of heated oil, a portion of which consists of partially polymerized oil and a further portion of which consists of completely polymerized oil, vaporizing said stream at such pressure and temperature that said completely polymerized oil remains liquid, all other portions including said partially polymerized oil being vaporous, said temperature and pressure being insufficiently high to cause gasoline formation but high enough to cause detrimental decomposition of said residue if continued, reducing the temperature of said residue to avoid such decomposition by introducing to the vaporizer a second oil, capable of being substantially completely vaporized at the temperature of said first vaporization, protecting said second oil from substantial contact with the vapors of said first vaporization, allowing said second oil to vaporize while in contact with said residue, admixing and simultaneously removing vapors from both vaporizations, and removing as a residue an oil sufficiently polymerized to have at least 60-70 per cent of 100 penetration asphalt and a relatively low content of material insoluble in carbon bisulphide.

4. That process of producing asphaltic residual oil which comprises establishing a stream of heated oil, a portion of which consists of partially polymerized oil and a further portion of which consists of completely polymerized oil, vaporizing said stream at such pressure and temperature that said completely polymerized oil remains liquid, all other portions including said partially polymerized oil being vaporous, said temperature and pressure being insufficiently high to cause gasoline formation but high enough to cause detrimental decomposition of said residue if continued, reducing the temperature of said residue to avoid such decomposition by introducing to the vaporizer a second oil, capable of being substantially vaporized at the temperature of said first vaporization, protecting said second oil from substantial contact with the vapors of said first vaporization, allowing said second oil to vaporize while in contact with said residue, admixing and simultaneously removing vapors from both vaporizations, diluting said residue with a predetermined unvaporized portion of said second oil, and removing as a residue an oil having at least 60-70 percent of 100 penetration asphalt and low in content of material insoluble in carbon bisulphide.

HENRY G. NEVITT.